

Patented Sept. 19, 1922.

1,429,503

# UNITED STATES PATENT OFFICE.

RUDOLF GRAEFFE, OF BRAND-ERBISDORF, NEAR FREIBERG, GERMANY.

## TREATING PEAT FOR MANUFACTURING AN INSULATING MATERIAL.

No Drawing.

Application filed January 6, 1921. Serial No. 435,567.

To all whom it may concern:

Be it known that I, RUDOLF GRAEFFE, a subject of Germany, and residing at Brand-Erbisdorf, near Freiberg, in Saxony, Germany, have invented certain new and useful Improvements in Treating Peat for Manufacturing an Insulating Material (Germany, G 48,717 VI/80<sup>b</sup>, 22nd July, 1919, Germany, G 49,491 VI/80<sup>b</sup>, Nov. 11th, 1919), of which the following is a specification.

This present invention relates to an improved treatment of peat for manufacturing a high-valued insulating material which by the special treatment hereinafter described is much improved with regard to the insulating material heretofore known consisting of a mixture of dried peat with a powdery binding substance which is put into heating drums or the like after being mixed in order to be melted. This process could not however provide a really valuable insulating material nor could this be obtained by mixing wet peat with respective binding substances on account of the great absorbing capacity of the peat, the latter always tending to regain its original degree of moisture, of which it had been deprived by drying or pressing, from the surrounding atmospheric air or the surrounding masonry and besides the peat having a liability to shrink and swell and thereby changing its volume, according to its being wet or dried which is a great disadvantage to its use as insulating material or the like.

Now the present invention is based upon the observation that in order to obtain a really good insulating material it is necessary to destroy the absorbing capacity of the peat and the shrinking and swelling qualities of the same, this being obtained by the present process in the most perfect manner as follows:—

Peat in any desired form and state, that is to say marshy or dried in pieces or reduced to fibres is boiled in water, whereby the marshy water may be used, and a tossing-tub or the like being adapted to thoroughly disintegrate the peat while boiling. After a boiling time of about one hour, in which time the peat deposits itself on the bottom of the boiler, coal-tar-pitch is put into the boiling peat, said pitch being in a state of foam by preheating the same to 200° C., whereby it will be observed that the coal-tar-pitch in this state is adapted to

thoroughly saturate the fibres of the peat which are completely dissolved by boiling. While the boiler is being filled with the foaming coal-tar-pitch the tossing-tub must be set at rest and will be actuated again, when all the coal-tar-pitch has been put into the boiler, the boiling process being simultaneously continued, whereby the coal-tar-pitch is homogeneously and thoroughly mixed with the peat-pulp. This is effected by the liquid pitch entering thoroughly into the dissolved fibres of the peat which are enlarged to their utmost volume by the boiling process, hereby bursting the wet walls of the cells and covering the fibres, inside and outside with a thin layer of pitch, whereby the foam forms a kind of medium, by which the coal-tar-pitch is introduced into the peat.

The effect of the process is as follows:—

(1) The perfectly even cover of the peat-fibres with a thin well-adhering layer of coal-tar-pitch forms after the solidifying fast but nevertheless elastic cover round each fibre which prevents the same from either swelling or shrinking.

(2) The destroying effects of the chemicals which were contained in the coal-tar-pitch on the slimy, swelled and colloidal substances of the fibres, taking from the same their water-absorbing qualities.

(3) The entrance of the finest parts of the coal-tar-pitch into the ends of the fibres, whereby in the solidifying of the coal-tar-pitch such a pressure is exercised upon the cells of said fibres that the same will presently burst, their capacity of absorbing water being destroyed in this way.

The finished pulp of peat and coal-tar-pitch may now be treated with respect to its further use as a simple filling-in or as insulating plates and forms. In the first instance the pulp may be dried on respective devices in any desired way, whereafter it is ready for use. In the second instance the finished mass is put into moulds of iron or the like as long as it is still hot and before being dried. These moulds being provided with walls which allow the water to escape whereafter the moulds brought under the influence of any desired pressure, that is to say steam or compressed air, whereby the water is withdrawn from the mass. Now the moulds are put into hand-or-hydraulic presses and the mass is reduced to about one half or one quarter of its previous vol-

- ume. As soon as these moulds hereby obtained are cooled they are ready for use. It is however advisable to store the same some short time before using in order that 5 the same may dry a little more, whereafter the moulds are still less liable to breakage and disforming by pressure or the like. The same are perfectly even and show the characteristics as cited above.
- 10 It is however possible to form the peat even after being dried in the above described manner, in wetting the same a little but not more than to about 25% of its dry-weight and only in such a manner that no 15 dust may rise in working the peat. This wet material is again filled into fast and well closed moulds and is reduced to about one third of its previous volume in heatable hand-or-hydraulic presses.
- 20 As in pressing the moulds of the peat-pulp the moulds used thereby are to be heated again to about 100° C., whereby a quick evaporation of the water which had been added to the peat before filling it into the 25 moulds is effected, which results in a chemical process very favourable to the pressing action and the peat retaining into once given form so that in a very few minutes a perfectly even and homogeneous body is 30 produced within the pressing forms.
- In order to obtain moulds of still greater firmness the peat may be mixed during its boiling process with a certain quantity of hot wet potter's clay or else, if the pressed 35 bodies must have a special resistance against heat, kieselguhr must be added besides such potter's clay.
- Finally the above described material may be used for manufacturing artificial stones 40 for building purposes in adding thereto cement, lime, gypsum or the like.
- It must be still observed that according to the above described invention a very valuable material is obtained. It may now 45 be possible that in certain instances a less valuable and therefore less expensive material may be used as well. In this case it is sufficient to add to the peat before boiling the same a well heated (unto 100° C.) quantity of coal-tar-pitch. By boiling both these 50 ingredients together a good mixture of the fibres and the pitch may be obtained though the same will be less even and perfect than the mixture according to the original form 55 of the present invention.
- A third possibility exists in preparing a still more valuable material than in the first named example by the peat being not only dessicated but roasted at a still higher 60 temperature and changed into coal, whereafter it may be treated as described in the
- first form of the process. Hereby a material is obtained which possesses quite an extraordinary insulating capacity against cold and heat, so that it may be used in special 65 cases. In further treating this material the mass may be filled into roasting pans instead of being simply dried after the mixing process and roasted therein in respective quantities. This repeated roasting may be 70 prolonged till the formation of coal, whereafter the roasted mass is filled into heatable presses in order to be pressed into moulds or like forms. It is evident that such forming may be done in the same time with the 75 aforesaid roasting process.
- It may be understood that all these different forms of the process of manufacturing an insulating material from peat in commingling it with coal-tar-pitch described 80 herein do not depart from the spirit of the present invention.
- Having now particularly described and ascertained the nature of my invention and in what manner the same is to be performed, I declare that what I claim is:—
1. The herein described insulating material composed of peat being boiled in water and coal-tar-pitch having been brought to foam by preheating to about 90 200° C. being mixed with said peat during the boiling process whereafter the thoroughly mixed material is dried and treated according to its further use that is pressed and formed into plates, substantially as 95 described.
2. The herein described insulating material composed of peat being boiled in water and coal-tar-pitch having been brought to foam by preheating the same to 100 about 200° C. being mixed with said peat thereto during the boiling process, whereafter the thoroughly mixed material is pressed in moulds while hot and before being dried, said moulds being brought under 105 the influence of steam or air under pressure whereafter the moulds are pressed in hand-or-hydraulic presses, substantially as described.
3. The herein described insulating ma- 110 terial composed of peat and coal-tar-pitch, said peat being roasted before its being boiled with the foaming coal-tar-pitch and the finished material being roasted again to turn into coal during its treatment in the 115 presses or moulds, substantially as described.
- In testimony whereof I affix my signature in presence of two witnesses.

RUDOLF GRAEFFE.

Witnesses:

Dr. LANDESKROENER,  
O. REINICKE.